

Patented Dec. 4, 1928.

1,693,640

# UNITED STATES PATENT OFFICE.

GEORGE E. DALBEY, OF EAST BERLIN, AND THOMAS P. HANFORD, OF BERLIN, CONNECTICUT, ASSIGNORS TO THE STANLEY CHEMICAL COMPANY, OF EAST BERLIN, CONNECTICUT, A CORPORATION OF CONNECTICUT.

## PROCESS FOR TREATING IMPURE LEAD.

No Drawing.

Application filed May 4, 1926. Serial No. 106,726.

This invention relates to a process for treating impure lead.

Impure lead usually contains one or more of the metals arsenic, tin and antimony. 5 These metals also exist as alloying matter in lead alloys and it is to be understood that the term impure lead includes lead alloys.

It is an object of the invention to provide an effective and economical process for treating 10 impure lead to remove arsenic, tin and antimony individually or collectively.

With this and other objects in view, the invention consists in the process which will first be described and then more particularly 15 pointed out.

Considering first, for convenience of description, the removal of tin from an alloy of tin with lead, in carrying out the process of the invention, the alloy is melted and is 20 treated in a molten condition in a receptacle suitably closed against an oxidizing atmosphere. Upon the molten alloy is placed a suitable amount of an oxide of lead, e. g. litharge. The contents of the receptacle are 25 stirred in any suitable manner and during this stirring there is slowly added upon the surface of the litharge and molten metal, a water solution of a caustic alkali, e. g. sodium hydroxide. It will be understood that this 30 slow addition of the caustic alkali referred to may be intermittent, the effect in view being a gradual addition rather than an abrupt addition of the entire batch.

As the water evaporates, the remaining sodium hydroxide becomes intimately mixed 35 with and reacts with the litharge. The stirring operation keeps the particles of litharge and resulting sodium plumbate separated into a fine state of division. It also continuously 40 brings the litharge, as it is being coated and treated with sodium hydroxide, into intimate contact with the molten metal. From a chemical standpoint, it is probable 45 that two reactions take place. First, the litharge is acted upon by the sodium hydroxide to form sodium plumbate. Secondly, a certain amount of tin is oxidized by the action of the litharge, the latter being reduced to metallic lead. There is also a 50 reaction between the tin oxide thus produced and the sodium hydroxide to form sodium stannate. Also, a reaction between the sodium plumbate and the tin in the molten alloy forms metallic lead and sodium stannate.

During the period of reaction, in carrying 55 out the process to the best advantage, the materials on the surface of the molten metal are maintained in a dry, powdery condition. In this way, avoiding the use of molten sodium hydroxide, the reaction is kept under proper 60 control and extremely beneficial results are obtained.

If desired, after a certain reaction period, the dry, powdery material may be removed 65 from the surface, a fresh batch of litharge provided, and a further reaction period carried out. The reaction may be accelerated by causing a portion of the molten alloy to be raised, for example, by a pump, and allowed to drop in globules onto and through 70 the superimposed litharge. This gives an intimate contact of the molten metal with the litharge and the sodium plumbate, or sodium hydroxide, as the case may be. The process described may be amplified in many ways, 75 e. g. by counter current operations in which the reagents and products of reaction may be removed from one receptacle and placed on molten metal in another receptacle.

In any event, when the reaction period is 80 continued for a sufficient time under proper conditions, substantially all the tin in the alloy is turned into sodium stannate, leaving the molten metal substantially free from tin.

During the evaporation of the water of 85 the sodium hydroxide solution, steam is formed in the closed receptacle and aids in preventing access of air to the materials undergoing reaction.

The process described is applicable to the 90 separation of arsenic and antimony from lead alloys. In the case of arsenic it is removed in the form of sodium arsenate and antimony is removed as sodium antimoniate.

In treating a lead alloy containing all 95 these metals, i. e. arsenic, tin and antimony, they may all be removed by the process described, in the order named. That is, there is a tendency toward the formation, first, of sodium arsenate, then sodium stannate and 100 lastly, sodium antimoniate. The tendency of the proportion at which one metal is removed in preference to another depends largely upon the ratio of amounts present to the total mass of molten metal. The reaction is allowed to 105 proceed to a certain point to remove substantially all the arsenic, then the powdery layer is removed and a fresh charge of litharge and

sodium hydroxide substituted. Another period of reaction is carried out, resulting in the removal of the tin. The powdery layer is again removed and another charge 5 of reagents supplied. The final period of reaction removes the antimony. Thus arsenic, tin and antimony are removed individually and separately from a lead alloy containing all these metals.

10 The above description sets forth the treatment of lead alloys. It will be understood that the treatment of impure lead is the same except that quantities may vary as in the case of impure lead the amounts of arsenic, 15 tin and antimony present are usually smaller than in the case of alloys. In either case metallic lead is reclaimed. In the case of alloys, where the amounts of alloying metals are substantial, there is also obtained one 20 or more alkali salts of such metals and these salts have commercial value.

What is claimed is:

1. The process of treating impure lead for the removal of arsenic, tin, antimony and the 25 like, which comprises bringing the metal in a molten condition under the influence of litharge and at the same time making gradual additions of a water solution of a caustic 30 alkali and maintaining the whole at a temperature which will always allow the reacting materials on the surface of the molten metal to remain in a powdery or granular condition.

2. The process of treating impure lead for 35 the removal of arsenic, tin, antimony and the like, which comprises bringing the metal in

a molten condition under the influence of an oxide of lead and at the same time making gradual additions of a water solution of a caustic alkali and maintaining the whole at 40 a temperature which will always allow the reacting materials on the surface of the molten metal to remain in a powdery or granular condition.

3. The process of treating impure lead for 45 the removal of arsenic, tin, antimony and the like, which comprises bringing the metal in a molten condition under the influence of litharge and at the same time making gradual 50 additions of a water solution of a caustic alkali and maintaining the whole at a temperature which will always allow the reacting materials on the surface of the molten metal to remain in a powdery or granular condition, and protecting the whole from an 55 oxidizing atmosphere.

4. The process of treating impure lead for the removal of arsenic, tin, antimony and the like, which comprises bringing the metal in a molten condition under the influence of 60 an oxide of lead and at the same time making gradual additions of a water solution of a caustic alkali and maintaining the whole at a temperature which will always allow the reacting materials on the surface of the 65 molten metal to remain in a powdery or granular condition, and protecting the whole from an oxidizing atmosphere.

In testimony whereof, we have hereunto set our hands.

GEORGE E. DALBEY.  
THOMAS P. HANFORD.